

## 1

2,889,223

STAINLESS STEEL ALLOY AND  
METHOD OF FORMING

Leroy E. Fink, Beaverton, and Raymond W. de Weese, Portland, Oreg., assignors to Electric Steel Foundry Company, Portland, Oreg., a corporation of Oregon

No Drawing. Application August 8, 1955  
Serial No. 527,168

4 Claims. (Cl. 75—130.5)

This invention relates to a stainless steel alloy, and more particularly to an alloy having an improved yield strength in the temperature range of 600° to 1200° F. and a proper impact resistance at room temperature, which alloy is readily weldable, easily machined, and has high corrosion resistance in the above indicated high temperature range. The alloy of this invention is particularly useful in producing castings which require unusual properties as to impact strength, corrosion resistance, weldability, etc.

Certain alloys having high corrosion-resistant properties have been heretofore suggested and are designated in A.C.I. Standard Designations (Alloy Casting Institute Standard Designations and Chemical Composition Ranges for Heat and Corrosion-Resistant Castings), one of such designations being ACI CF-3M. Similar designations, showing comparable compositions, are set out in the well-recognized AISI-T318, and more particularly in AISI Type 316, AISI Type 317 and AISI Type 318. It has been suggested in some studies relating to the production of elevated temperature corrosion resistant castings that an alloy be obtained with a small percentage of ferrite in the as-cast condition, heat-treating the alloy at 2050° F. for 4 hours to place all carbides in solution, water quenching to keep them in solution, maintaining the material for 5 hours at 1550° F., and then cooling in still air to transform the small percentage of ferrite into sigma phase. The results showed tensile values determined at 700° F. lower than the desired 25,000 p.s.i.

In the foregoing work, it was discovered that considerable difficulty was encountered in attempting to maintain the ferrite content at 5-10%. Such a ferrite content was desired to give the desired weldability. The lower the ferrite content, the more difficult it is to weld without encountering hot shortness. On the other hand, as the ferrite content is lowered, the impact values improve. To produce a product meeting the critical requirements above outlined, it is desirable to maintain the ferrite content between 5 and 10%.

We have discovered that an alloy can be produced meeting the extreme requirements heretofore set out by employing a chemical range or composition which will be hereinafter set out, and thereafter, in the treatment of the starting materials, making tests at the furnace itself and adding the necessary alloys to the bath to bring the bath to the proper ferrite range. In this process, the chemical range of the ingredients plays an important part, as will be set out more fully hereinafter.

An object of the present invention is to provide a simple and effective process whereby a stainless steel alloy having the critical and high requirements heretofore stated may be obtained in regular plant operation. Another object is to provide a formula or chemical range which is effective in the carrying out of the process for producing the new alloy. A still further object is to provide a chemical range and method for producing an alloy having an improved yield strength in high temperature ranges, good impact resistance at room temperature,

## 2

excellent corrosion resistance at high temperatures, while being readily weldable and easily machined. Other specific objects and advantages will appear as the specification proceeds.

5 In one embodiment of our invention, we form a bath in a furnace such as an electric furnace, containing the following chemical ingredients:

|            |               |
|------------|---------------|
| Chromium   | 17.25-18.25%. |
| 10 Nickel  | 12.00-13.00%. |
| Carbon     | 0.034% max.   |
| Molybdenum | 2.25-3.00%.   |
| Silicon    | 0.35-0.75%.   |
| Manganese  | 1.0% max.     |

15 Columbium and tantalum 10 times carbon content.

Any suitable procedure in the combining of the elements in the bath may be employed. By way of example, the charge may consist of clean mild steel, nickel,

20 and molybdenum, which may be melted down in a basic-lined arc furnace until the bath reaches a temperature in the neighborhood of 3000° F. Treatment with lime and with oxygen may follow, and after the boil, ferrosilicon and ferrochromium may be added. Later lime may be added again and low carbon ferromanganese and ferro columbium-tantalum. A sample may be taken for carbon determination. To build up the silicon and chromium contents to the desired level, selected amounts of ferrochromium, ferrosilicon and ferro-chromium-silicon may be used.

30 In order to determine the ferrite content, a series of samples are taken and the magnetic permeability of each sample determined by a standard permeability tester. The necessary alloys are then added to the bath to bring the bath to the proper ferrite range. The method of making the ferrite test is described in greater detail in the copending application of Leroy E. Fink, Serial No. 499,765, now abandoned.

35 The embrittlement or cracking tendency of the alloy known as "hot shortness" may further be combated by adding to the metal vanadium and titanium and also, if desired, a small amount of boron. It is preferred to add the titanium in the amount of 0.01 to 0.06% and the vanadium in the proportion of about 0.02 to 1%. Very good results are obtained when the vanadium and titanium are added in the proportions of 0.05 to 0.25% vanadium and 0.01 to 0.15% titanium. A more complete description of the addition of such metals to combat hot shortness is set forth in the copending application of Leroy E. Fink, Serial No. 485,341, now abandoned. It will be understood that the adding of the vanadium, titanium and boron is an optional procedure and may be omitted, if desired.

40 It is also possible to produce the desired alloy using columbium alone, and without tantalum, at eight times the carbon content, and the ranges may be set out as follows:

|            |               |
|------------|---------------|
| Chromium   | 17.25-18.25%. |
| 60 Nickel  | 12.00-13.00%. |
| Carbon     | 0.034% max.   |
| Molybdenum | 2.25-3.00%.   |
| Silicon    | 0.35-0.75%.   |
| Manganese  | 1.0% max.     |
| Columbium  | 8-10×carbon.  |

45 65 We have discovered that within the ranges set out above and on column 2 lines 9-15 hereof, the desired product can be produced if the ferrite content in the final alloy is kept at 5-10%. We have found that the lower the ferrite content, the more difficult to weld without encountering hot shortness, while with a lowered ferrite content, the impact values improve. By maintaining the

ferrite content in the range of 5-10%, the ranges described in the foregoing tables may be effectively employed in producing the important new alloy. Various tests may be employed in determining the ferrite content during the progress of the operations, as, for example, the employment of the magnetic permeability test referred to above, or by employing other suitable test methods. By utilizing the ranges described and adding the necessary ingredients to maintain the ferrite content of 5-10%, a highly successful result is achieved.

In the production of the metal alloy, it is the chemical composition of the alloy that determines the phase or crystal structure of the solid metal, and in the practice of the present invention, we find that it is desirable to obtain a rough control of the composition and characteristics of the alloy product by combining the alloying materials in predetermined proportions as set out in the above preferred chemical ranges, modifying the composition as later determined by the tests made at the furnace to give the desired product having the ferrite content of 5 to 10%. The added materials are austenite-formers and ferrite-formers having different grades of potency. For example, molybdenum, silicon, chromium and columbium are ferritizers, while nickel, carbon, and manganese are austenitizers. Well known formulas indicate the potency of these elements, and the elements may be added to bring about the desired chemical composition as the magnetic permeability tests are made. In making the tests at the furnace, a sample is withdrawn and solidified and the magnetic permeability measured by a standard instrument such as, for example, the permeability tester produced by the Severn Engineering Company, of Annapolis, Maryland. Next, the measured value of the magnetic permeability of the sample is compared with a previously established standard value corresponding to the pre-selected proportions of magnetic and non-magnetic components, the magnetic component being ferrite and the nonmagnetic component being austenite. Next, a metal alloying material is added, and this is either a material which has the property of increasing, or a material which has the property of decreasing, the relative proportions of magnetic to nonmagnetic components in the metal alloy. It is usually necessary to repeat the steps a number of times until the last measured value for magnetic permeability closely approximates the standard value, thereby indicating that the pre-selected proportions of magnetic and nonmagnetic components have been achieved and more particularly bringing the ferrite content within the selected range of 5 to 10%.

For the effective operation of the process, we found that the chemical range heretofore set out provides the rough control which is necessary and effective for producing the new alloy, and in this chemical range the

The following specific examples may be set out as illustrative:

#### Example I

The charge consisting of clean mild steel, nickel and molybdenum is melted down in a basic lined arc furnace until the temperature of the bath reaches 2950-3000° F., after which lime is added. In this example, a "Electromelt," size PT, furnace was employed. Following this, the electrodes and roof are lifted and the heat is boiled with oxygen for a predetermined time depending on charge weight. After the boil, 75% ferro-silicon and Simplex ferrochromium are added. The power is then switched to #1 tap which was set for 9000 amperes at 215 volts. When the Simplex ferrochrome is almost melted, the balance of the lime is added and the power is switched to #2 tap which was set for 8800 amperes at 185 volts. Then, when the lime is completely melted, extra low carbon ferromanganese and ferro columbium-tantalum is added. A spoon sample is taken for carbon determination. (The power is turned off while the carbon is determined and resumed immediately after the determination is made.) To build up the silicon and chromium contents to the desired level, selected amounts of ferrochromium, 50% ferrosilicon and ferrochromium-silicon are used for this purpose.

When homogeneity is achieved and the heat is ready to be tapped, a sample is taken with a slagged spoon and poured into a copper mold. The metal is allowed to cool in this mold until black. It is then removed and quenched in water. When cool, the bottom surface of the sample is tested with a Severn Engineering Company Permeability Tester. Depending on the results of this test, small amounts of alloy agents (e.g., chromium, nickel, manganese, silicon) may be added to adjust the chemical composition to obtain the desired ferrite content. After any addition is made to the molten bath in the furnace, the metal is well stirred to obtain a homogeneous bath. Another sample is then taken. This procedure is continued until the desired ferrite content, as determined by magnetic permeability, is obtained. When this occurs, the temperature of the bath is determined and if the temperature is 3200° F., or greater, the heat is tapped.

#### Example II

A series of examples is illustrated by the following table setting forth end analyses and physical properties of the castings obtained. The castings have the necessary physical properties and are weldable. The analyses demonstrate the interaction of the elements themselves on the ferrite constituent while ferrite-forming chromium is balanced off by austenite-forming nickel, carbon or manganese.

| Heat No. | Chemical Composition, percent |     |     |       |       |      |     |      |      | Tensile Strength, p.s.i. | Mechanical Properties               |                       |                         | BHN | Impact in ft.-lbs., Charpy Keyhole | Yield Strength, p.s.i. at 700 F. |
|----------|-------------------------------|-----|-----|-------|-------|------|-----|------|------|--------------------------|-------------------------------------|-----------------------|-------------------------|-----|------------------------------------|----------------------------------|
|          | C                             | Mn  | Si  | Cr    | Ni    | Mo   | Cb  | S    | P    |                          | Yield Strength, 0.2% offset, p.s.i. | Elong. in 2", percent | Reduc. in Area, percent |     |                                    |                                  |
| 44-163   | .028                          | .79 | .66 | 18.20 | 12.42 | 2.39 | .27 | .023 | .023 | 77,500                   | 48,500                              | 40                    | 41.6                    | 170 | 25, 26, 43                         | 28, 250                          |
| 44-159   | .031                          | .52 | .72 | 18.12 | 12.27 | 2.53 | .24 | .020 | .023 | 73,000                   | 44,000                              | 48                    | 48.6                    | 163 | 19, 28, 43                         | 25, 250                          |
| 44-168   | .032                          | .86 | .80 | 18.18 | 12.41 | 2.43 | .27 | .019 | .023 | 72,000                   | 40,000                              | 52                    | 51.7                    | 170 | 20, 35, 38                         | 25, 500                          |
| 44-171   | .023                          | .61 | .56 | 17.95 | 12.80 | 2.35 | .27 | .020 | .021 | 76,500                   | 47,500                              | 38                    | 54.9                    | 170 | 18, 20, 42                         | 33, 600                          |
| 44-174   | .030                          | .52 | .48 | 18.18 | 12.71 | 2.51 | .20 | .024 | .020 | 79,000                   | 52,500                              | 39                    | 45.8                    | 187 | 26, 28, 46                         | 33, 750                          |
| 44-176   | .021                          | .71 | .57 | 18.32 | 12.70 | 2.53 | .27 | .012 | .019 | 79,000                   | 52,000                              | 41                    | 41.6                    | 170 | 19, 25, 48                         | 26, 500                          |
| 44-167   | .030                          | .78 | .78 | 17.82 | 12.17 | 2.50 | .26 | .022 | .023 | 75,000                   | 42,500                              | 47                    | 45.5                    | 156 | 19, 26, 34                         | 27, 600                          |

chromium may be from 17.25 to 18.25%. The nickel may be 12.00 to 13.00%, the carbon should be 0.034% maximum, and the molybdenum 2.25-3.00%. The silicon should be 0.35-0.75%, and the manganese 1.0% maximum. The columbium plus tantalum should be 10 times the carbon content.

While, in the foregoing specification, we have set forth specific ranges and analyses and steps of procedure in considerable detail for the purpose of illustrating the invention, it will be understood that such details may be varied widely by those skilled in the art without departing from the spirit of our invention.

We claim:

1. In a method of producing a stainless steel alloy having a pre-selected proportion of ferrite, the steps of combining with steel in a molten bath and in the proportions indicated, chromium 17.25-18.25%, nickel 12.00-13.00%, carbon 0.034% maximum, molybdenum 2.25-3.00%, silicon 0.35-0.75%, manganese 1.0% maximum, and columbium plus tantalum 10 times the carbon content, drawing samples from the bath and determining the ferrite content thereof, and adding to the same molten bath an alloy material selected from the group consisting of ferrite-formers and austenite-formers to bring the ferrite content between 5 and 10%.

2. The process of claim 1, in which the ferrite content is determined by determining the magnetic permeability of the withdrawn bath sample.

3. The process of claim 1, in which a small percentage of titanium and vanadium are added, the vanadium being in the range of 0.02 to 1% and the titanium being in the range of 0.01 to 0.06%.

4. In a process for producing a readily-weldable stainless steel alloy of high impact resistance at room temperature, the steps of combining with steel in a molten bath, and in the proportions indicated, chromium 17.25-18.25%, nickel 12.00-13.00%, carbon 0.034% maximum, molybdenum 2.25-3.00%, silicon 0.35-0.75%, manganese 1.0% maximum, and columbium 8 to 10 times

the carbon content, periodically drawing molten samples from the bath and determining the ferrite content thereof, adding to the same molten bath alloy materials selected from the group consisting of ferrite-formers and austenite-formers to bring the ferrite content between 5 and 10%, and then pouring the molten metal.

References Cited in the file of this patent

UNITED STATES PATENTS

|           |                |       |               |
|-----------|----------------|-------|---------------|
| 2,159,724 | Franks         | ----- | May 23, 1939  |
| 2,240,672 | Scherer et al. | ----- | May 6, 1941   |
| 2,481,386 | Bloom          | ----- | Sept. 6, 1949 |
| 2,544,336 | Linnert        | ----- | Mar. 6, 1951  |

OTHER REFERENCES

Transactions, American Society for Metals, vol. 39, 1947, pages 868 to 871. Published by the A.S.M., Cleveland, Ohio.

20 Buck et al.: ASTM Symposium on Evaluation Tests for Stainless Steels, 1950, Special Tech. Publ. No. 93, pages 56-86. Published by the American Society for Testing Materials, Philadelphia, Pa.

25 Binder et al.: ASTM Symposium on Evaluation Tests for Stainless Steels, 1950, Special Tech. Publ. No. 93, pages 146-182. Published by the American Society for Testing Materials, Philadelphia, Pa.